

A. L. MARSH.  
METAL UTENSIL.  
APPLICATION FILED JAN. 19, 1917.

1,229,770.

Patented June 12, 1917.



Witnesses:

John Taylor.

Irvin Bowman.

Inventor:

Albert L. Marsh,  
By appointment of the  
Inventor, *Albey*

# UNITED STATES PATENT OFFICE.

ALBERT L. MARSH, OF DETROIT, MICHIGAN, ASSIGNOR TO HOSKINS MANUFACTURING COMPANY, OF DETROIT, MICHIGAN, A CORPORATION OF MICHIGAN.

## METAL UTENSIL.

1,229,770.

Specification of Letters Patent. Patented June 12, 1917.

Application filed January 19, 1917. Serial No. 143,369.

To all whom it may concern:

Be it known that I, ALBERT L. MARSH, a citizen of the United States, residing at Detroit, in the county of Wayne and State of Michigan, have invented a new and useful Improvement in a Metal Utensil, of which the following is a specification.

My invention relates to certain new and useful improvements in a metal utensil of the character which is exposed in use to the destructive action of molten brasses, bronzes and the like, and is fully described and explained in the specification and shown in the accompanying drawings, in which:

15 Figure 1 illustrates the application of my invention to a thermo-couple; Fig. 2 to a thermo-couple protecting tube; and Fig. 3 to a crucible.

Many efforts have been made to make a thermo-couple, or thermo-couple protecting tube, for use in measuring the temperature of molten metal, particularly brass, at relatively high temperatures. Many experiments with materials of various kinds have 20 been made in an effort to attain this end, but the materials heretofore employed have proved unsatisfactory in practice, owing to their rapid disintegration under the conditions of use. I have discovered, however, 25 that an alloy of iron and chromium is entirely satisfactory for this purpose.

In use in the ordinary bath of brass there are two wholly different conditions tending to destroy the protecting tube or any other 30 metal entering the bath. There is, in the first place, the solvent action of the brass which tends to disintegrate that part of the metal element which is immersed. The metal element above the bath line is 35 naturally highly heated, and the atmospheric oxygen tends to attack this part of the metal article and destroy it with considerable rapidity. I have shown in a previous patent (Number 1057754) that an alloy of iron and chromium is highly resistant to oxidation (at least under the high 40 temperature to which electric heating elements are subjected) when the chromium is upward of 20 per cent., the resistance to oxidation being very high at about 25 per cent. chromium. The alloys of chromium and iron, beginning at about 15 per cent. chromium, are highly resistant to the dissolving action of the brass bath, but I prefer to use for most purposes an alloy con-

taining approximately 25 per cent. chromium in order to get also the high resistance to oxidation at the high temperatures commonly employed in brass melting. However, with various brasslike alloys which melt at lower temperatures than ordinary brass the importance of resisting oxidation is smaller and the alloys lower in chromium can be profitably employed.

I also find that while not necessary, the addition of about 2 per cent. of manganese to the alloy renders the alloy less soluble in certain grades of brass, although it seems to be without effect in others. The preferred alloy, therefore, for the manufacture 60 of the articles forming the subject-matter hereof consists of 25 per cent. chromium, 75 per cent. iron, with an addition of 2 per cent. manganese.

It will be perfectly evident to those skilled in alloys that other ingredients can be added, possibly in considerable quantities, to the present alloy without materially interfering with the operative qualities of the articles made therefrom.

My first embodiment of the present invention in a concrete structure is that illustrated in Fig. 2, where I have shown an ordinary thermo-couple protecting tube formed of my preferred alloy, a thermo-couple of the ordinary form being located within the same. This protecting tube can be partially immersed in a bath of molten brass for long periods of time without serious disintegration and affords the first 75 commercial and successful means for applying the thermo-couple measurements to brass melting.

In Fig. 1, I have shown a device in which one element of the thermo-couple and the protecting tube are combined into a single piece, the other element of the thermo-couple passing down centrally within the tube and being welded to its bottom. The millivoltage temperature curve of my preferred alloy is of a highly satisfactory form, thereby adapting the material for convenient thermo-couple use in connection with a standard meter. The millivoltage is not high and by selecting either a strongly negative or strongly positive material this alloy can be used either as a positive or negative element. For instance, my present preferred alloy when used with a nickel chromium element is positive and when used with 80 85 90 95 100 105 110

a nickel aluminum element is negative, considering the direction of electrical flow at the hot junction, the element to which the current flows from the hot junction being 5 negative.

I have further discovered that precisely the same qualities which render this alloy suitable for the manufacture of protecting tubes, and which render the thermo-couple 10 of Fig. 1 durable, makes it possible to construct a large number of novel and highly desirable devices therefrom, all of which depend for their enhanced usefulness upon the resistance of the alloy both to oxidation 15 and to the dissolving effect of molten brass and similar metal baths. For instance, melting crucibles, such as that shown in Fig. 3, when made of this alloy are found to be highly durable, comparing favorably with 20 plumbago crucibles, and in use, even at high temperatures, they are much less fragile, and the relatively high thermal conductivity permits much more rapid melting and economizes fuel. Manifestly, also, the 25 present crucible absorbs no moisture when idle, and therefore requires no preliminary heating, such as is common practice with plumbago crucibles.

The same properties of the alloy adapt it 30 to the manufacture of other utensils or articles which in practice are brought into contact with the destructive influence of molten or highly heated metals, such as brass. Among such articles may be mentioned 35 dies, dies for die-casting, stirring rods, etc.

I have tested this alloy to confirm its resistance to the destructive influences not only of standard brass but of a large variety of bronzes, and I find that the articles 40 made therefrom are highly durable under all the conditions to which it has been subjected.

I realize that considerable variation is 45 possible in the details of this construction without departing from the spirit of my invention; therefore I do not intend to limit

myself to the specific form herein shown and described except as pointed out in the following claims, in which it is my intention to claim all the novelty inherent in the 50 construction as broadly as is permitted by the state of the art.

What I claim as new and desire to secure by Letters Patent is—

1. As an article of manufacture a metal 55 utensil of the character which is exposed in use to the destructive action of molten brasses, bronzes and the like formed of an alloy comprising iron and chromium.

2. As an article of manufacture a metal 60 utensil of the character which is exposed in use to the destructive action of molten brasses, bronzes and the like formed of an alloy comprising iron and upward of 15 per 65 cent. chromium.

3. As an article of manufacture a metal utensil of the character which is exposed in use to the destructive action of molten brasses, bronzes and the like formed of an alloy comprising iron and approximately 25 70 per cent. chromium.

4. As an article of manufacture a metal utensil of the character which is exposed in use to the destructive action of molten brasses, bronzes and the like formed of an 75 alloy comprising iron, chromium and a relatively small percentage of manganese.

5. As an article of manufacture a metal utensil of the character which is exposed in use to the destructive action of molten 80 brasses, bronzes and the like formed of an alloy comprising iron, upward of 15 per cent. chromium and a relatively small percentage of manganese.

6. As an article of manufacture a metal 85 utensil of the character which is exposed in use to the destructive action of molten brasses, bronzes and the like formed of an alloy comprising iron, approximately 25 per cent. chromium and approximately 2 per 90 cent manganese.

ALBERT L. MARSH.